

April 23, 1935.

W. B. LOGAN

1,998,765

PROCESS FOR NEUTRALIZING ORGANIC ACIDITY IN PETROLEUM LUBRICATING OILS

Filed Oct. 8, 1931



WILLIAM B. LOGAN

INVENTOR

BY *R. J. Dearborn*  
HIS ATTORNEY

## UNITED STATES PATENT OFFICE

1,998,765

PROCESS FOR NEUTRALIZING ORGANIC  
ACIDITY IN PETROLEUM LUBRICATING  
OILSWilliam B. Logan, White Plains, N. Y., assignor to  
The Texas Company, New York, N. Y., a corporation of Delaware

Application October 8, 1931, Serial No. 567,535

3 Claims. (Cl. 196—35)

This invention relates to the manufacture of lubricating oils and more particularly to a process of obtaining lubricating oils in improved form from crude petroleum.

5 The invention contemplates improvements in the manufacture of hydrocarbon lubricating oil from crude petroleum especially from crudes of the naphthene and mixed base types. The invention comprises preparing a lubricating oil containing fraction from the crude, and treating the fraction with an alkaline material during heating in the liquid phase to effect chemical reaction between the alkaline material and the acidic constituents of the oil, following which the oil is 10 subjected to distillation, preferably under subatmospheric pressure, for the production of desired lubricating oil fractions free from naturally-occurring and other acidic constituents.

According to my invention, crude oil is charged 20 to a pipe still or other suitable distilling means which may be adapted to operate at atmospheric pressures and wherein the gasoline, kerosene and the larger portion of the gas oil constituents of the crude are removed. The remaining or residual portion of the crude containing the lubricating fractions may constitute the fraction undergoing treatment according to my invention. On the other hand, a distillate lubricating oil fraction intermediate between the gas oil and the 25 residual or fuel oil portion of the crude may be prepared, advantageously, by subjecting the topped crude to distillation under subatmospheric pressure.

The resulting lubricating oil distillate or topped 30 crude, as the case may be, is mixed with strong alkali solution in suitable mixing or contacting means adapted to finely disperse the solution throughout the body of oil and the mixture then passed through heating coils wherein it is digested while maintained in substantially the 35 liquid phase during heating up to temperatures corresponding substantially to the distilling temperature of the oil at pressures less than atmospheric. The temperatures prevailing during 40 passage of the mixture through the heating coil may range from 100° F. to around 700° F. or even higher, depending upon the nature of the oil undergoing treatment, while pressures of around 100 pounds or at least sufficient to prevent substantial 45 vaporization of the oil as well as of the alkali solution may be impressed upon the mixture while passing through a considerable portion of the coil so as to maintain suitable and effective conditions of digest during a sufficient period of time.

50 The digested and heated mixture is then sub-

jected to distillation under subatmospheric pressure conditions, and while still in the presence of the alkali material to produce the desired lubricating oil fractions free from organic acids. The vacuum distillation may be carried out either 5 in a plurality of shell stills from each of which a desired vapor fraction is removed, or in a dephlegmating or flash column from which a plurality of liquid streams, each of desired viscosity characteristic, may be withdrawn at successive 10 points in the column. The vacuum distilling system is maintained under a low absolute pressure, preferably not in excess of about four or five inches of mercury, while the temperature of the oil may range from around 400 to not greatly 15 in excess of about 700° F. or 750° F.

In the prior art where oil has been distilled in the presence of caustic or other alkaline materials, it has been the practice to introduce the alkali directly into the still in which distillation 20 occurs. When alkali in the form of an aqueous solution is introduced into the hot still in this way, the aqueous portion thereof is immediately and instantaneously flashed into vapor, whereupon the alkali salt tends to settle out of the oil 25 on to the still bottoms. Thus a relatively large proportion of the oil is vaporized within the still without making any appreciable contact with the alkali, while the unvaporized portion of the oil makes scarcely any more contact with the 30 salt due to the rapidity with which the solid material settles out. The result is that there is scarcely any opportunity afforded for the alkali to react with the acidic constituents of the oil. These acidic constituents, particularly the naturally-occurring constituents, such as naphthenic 35 acids and the like, require prolonged and intimate contact with the alkali at elevated temperatures in order to completely react therewith. The necessary contact between alkali and oil is realized only when it is maintained in contact with the oil in the form of an aqueous solution; otherwise, as has been the case hitherto, the reaction 40 is far from complete and the resulting vaporized oil has contained large amounts of undesired 45 acidic material.

In certain instances, the treatment of hydrocarbon oils with caustic or alkali has, in the past, been restricted to a rather secondary or final operation, usually following acid treatment of the 50 oil. The alkali material has been immediately separated from the oil and the oil then usually washed with water to remove last traces of the caustic before undergoing any further treatment.

55 I have discovered that by digesting lubricating

- oil distillate with caustic soda or other suitable alkali material in aqueous solution at substantially the distilling temperature of the oil but while maintaining the oil in liquid phase and then 5 without removing the caustic or caustic reaction products, immediately subjecting the oil to distillation into desired fractions or cuts, and while still in the presence of the caustic an improved product results. The resulting product is of such 10 quality that acid treatment may be entirely omitted if desired.

The operation of the invention will now be described in connection with the accompanying flow diagram showing one form of apparatus 15 suitable for carrying out the invention.

Lubricating distillate or topped crude, as the case may be, is drawn either from a storage tank 1 or directly from distilling means and delivered through a pipe 2 to a mixer 3 wherein the oil 20 is brought into intimate contact with alkali solution. The alkali solution, which may comprise caustic soda of from 30° to 40° Bé. gravity, is introduced to the mixer from a storage tank 4 by a suitable proportioning pump 5. The mixer may 25 consist of a closed drum containing packing material jet or baffles, or may comprise any other suitable type of mixing means adapted to uniformly and finely disperse the alkali solution throughout the body of the oil.

30 The mixture of oil and alkali solution is passed from the mixer through a pipe 6 to a pipe coil heater 7 advantageously of the single continuous tubular type wherein the oil is maintained in turbulent flow during passage therethrough so as 35 to maintain the alkali solution and oil in an intimate state of admixture and thus avoid the separation of the alkali from the oil. The coil is preferably of such type that the mixture may traverse a distance of several thousand feet under 40 highly turbulent conditions of flow and under conditions of pressure and temperature such that the alkali solution is advantageously maintained in substantially a liquid phase so as to facilitate more effective contact with the oil. During flow 45 through the remaining portion of the coil, the mixture is subjected to still higher temperatures and passes through a zone wherein it may be largely vaporized.

In the case of a lubricating distillate fraction, the oil and alkali mixture may be heated to temperatures up to from 500 to about 700° F. while in the case of a heavier residual fraction, the temperatures may be around 750° F. or even higher. Thus, the mixture of oil and alkali is 55 subjected to heating at elevated temperatures to effect reaction between the alkali and the acidic constituents of the oil, preferably while maintaining the oil in a substantially liquid phase condition. By maintaining rapid and turbulent 60 flow of the liquid through the heating coil, subjection of the oil to cracking conditions for appreciable periods of time is avoided.

The pressure at the outlet of the coil may be 65 maintained at atmospheric pressure or thereabouts but may be less than atmospheric at this point as already set forth, the extent of such pressure being controlled by means of a control valve 8 located in the discharge pipe 9 from the heater 7. The heated mixture of oil and alkali, 70 after passage through the valve 8, is introduced to a dephlegmating column 10 maintained under a low absolute pressure, preferably not in excess of about two or three inches of mercury.

The oil is flashed into vapor in the lower portion 75 of the column and the vapors as they rise

towards the top of the column are subjected to fractionation and partial condensation into desired fractions which are withdrawn as side streams from the column.

Steam may be introduced to the bottom of the column 10 through a spray 11 for the purpose of 5 facilitating the vaporization of the oil. Reflux or cooling liquid may be introduced to the top of the fractionator through a spray 12 to supply the necessary cooling thereto so as to control the 10 degree of condensation. The desired lubricating oil fractions are removed as side streams from the fractionator through pipes 13, 14, etc.

The remaining uncondensed and gaseous material, including water vapor, is removed from 15 the top of the fractionator through pipe 15 to a barometric condenser 16 wherein it is contacted with cooling water admitted to the barometric condenser through a pipe 17. The fixed 20 gases and other incondensable material accumulating in the barometric condenser are removed therefrom through a pipe 18 to a vacuum pump 19 from which they may be exhausted to the atmosphere and by which means the desired degree of vacuum is maintained on the column 21. 25

The residual matter collecting in the bottom of the column 10, composed of tarry constituents together with the caustic reaction products, is withdrawn therefrom through a cooling 30 worm 20 from which it may be conducted to tankage.

It is contemplated that the temperatures and pressures described in connection with the foregoing example may be varied as desired, depending on the nature of the oil undergoing 35 treatment. The invention may be readily adapted to the treatment of various distillates or residual fractions derived from different crude sources, such as naphthene or mixed base crudes, as may be obtained from Gulf Coastal and Mid- 40 continent fields.

Obviously many modifications and variations of the invention, as hereinbefore set forth, may be made without departing from the spirit and scope thereof, and therefore only such limitations should be imposed as are indicated in the 45 appended claims.

I claim:

1. The method of simultaneously separating heavy residual petroleum lubricating oil stock 50 into lubricant distillate fractions while removing the naturally occurring acids therefrom, which comprises admixing the oil stock with a concentrated aqueous caustic soda solution, flowing the mixture in a confined turbulent stream through 55 a heating coil and rapidly heating it to a temperature of around 750° F. or higher while under sufficient pressure to maintain in substantially the liquid phase, flashing the heated mixture without previous removal of water vapor directly into an intermediate portion of a fractionating zone maintained under high vacuum, passing unvaporized oil downwardly through a lower portion of the fractionating zone and subjecting it therein to further distillation, fractionating the vapors to condense a lubricant fraction in the fractionating zone, removing such lubricant fraction as a side stream from the fractionating zone, and removing water vapor and remaining vaporized constituents overhead 70 from the fractionating zone.

2. The method of simultaneously separating heavy residual petroleum lubricating oil stock into lubricant distillate fractions while removing the naturally occurring acids therefrom, which 75

comprises admixing the hydrocarbon oil with an excess of a concentrated aqueous caustic soda solution, flowing the mixture rapidly in a confined turbulent stream through a heating coil and rapidly heating it to a temperature of around 750° F. or higher while under sufficient pressure to maintain in substantially the liquid phase, flashing the heated mixture without previous removal of water vapor directly into an intermediate portion of a fractionating zone maintained under high vacuum, passing unvaporized oil downwardly through a lower portion of the fractionating zone countercurrent to steam to effect further distillation thereof, fractionating the vapors to condense lubricant fractions in the fractionating zone, removing such lubricant fractions as side stream from the fractionating zone, removing water vapor and unvaporized constituents overhead from the fractionating zone, and removing residuum from the lower portion of the fractionating zone.

3. The method of simultaneously separating heavy residual petroleum lubricating oil stock into lubricant distillate fractions while removing the naturally occurring acids therefrom, which comprises admixing the oil stock with a concentrated aqueous caustic soda solution, flowing the mixture in a confined turbulent stream through a heating coil and rapidly heating it to a temperature of around 750° F. or higher while under sufficient pressure to maintain in substantially the liquid phase, flashing the heated mixture without previous removal of water vapor immediately into a fractionating zone maintained under high vacuum, passing unvaporized oil downwardly through a lower portion of the fractionating zone and subjecting it therein to further distillation, and fractionating the vapors to condense a lubricant distillate fraction substantially free from organic acidity.

5

10

15

20

WILLIAM B. LOGAN.